

# UNITED STATES PATENT OFFICE.

JOHN COTTER PELTON, OF SAN FRANCISCO, CALIFORNIA.

## PROCESS OF MAKING COLORED SAND.

1,233,501.

Specification of Letters Patent. Patented July 17, 1917.

No Drawing.

Application filed July 19, 1915. Serial No. 40,654.

To all whom it may concern:

Be it known that I, JOHN COTTER PELTON, a citizen of the United States, residing at San Francisco, in the county of San Francisco and State of California, have invented a new and useful Process of Making Colored Sand, of which the following is a specification.

This invention relates to the preparation 10 of sand for use in building construction, for example, as an aggregate or ingredient for mortar, cement, plaster, roofing paper, etc., and the primary object of the invention is to provide material of this character which 15 will enable any desired shade of building stone, block, mortar and roofing paper to be produced without the mixture of extraneous coloring matter.

Another object of this invention is to provide 20 for permanency and greater uniformity, intensity and brilliancy in the coloring of the sand than is possible with the processes heretofore known.

A further object is to so treat the grains 25 of sand that the coloring matter will be enabled to penetrate into the interior of said grains to a maximum degree.

A further object is to provide a process 30 in which the coloring is fixed in the sand and is not liable to wash out or fade.

Other objects of the invention will appear hereinafter.

In carrying out my invention, sand to be colored is first treated to widely different 35 degrees of temperature and to effect this the grains of sand are burned or heated red hot and while hot are suddenly cooled or given a cold fluid bath. The heat causes the grains of sand to expand and the fissures 40 and pores therein to enlarge and when the heated sand is suddenly cooled the shock or sudden change of temperature causes the grains to contract quickly thus setting up internal stresses and strains so that the 45 grains crack and partly break and become irregular in contour, thus making it more susceptible to penetration by coloring matter and more capable of holding the color. Sand treated in this way is improved in 50 quality for cement work and the like, as the jagged or rough nature of the grains conduces to greater adhesion between the grains and the cement particles.

The cold bath may also constitute the coloring 55 bath and if the coloring is to be effected in this way a coloring agent or agents

for imparting color to the sand or imparting the appearance of color to the sand is dissolved or suspended in a suitable solvent or medium such as cold water. After the 60 preliminary heating the sand may be thrown into the cold color bath so that the coloring matter will immediately enter into the fissures and pores of the grains of sand.

Or, if desired, the color bath may be a 65 separate step from the cooling treatment and follow the cold treatment.

The coloring agents which I have successfully employed consist of any suitable coloring-producing metallic salts or compounds.

The nature of the agent depends upon the color which is to be given the sand, and I apply this metallic matter to the sand in the form of a solution while it is dissolved 75 or suspended in a suitable solvent or carrying medium, the sand being soaked or impregnated with such solution or medium carrying the coloring matter.

The fissures and crevices become filled 80 with the coloring matter which is retained by the sand in this way. The sand is dried next and burned or heated again to intensify and aid in setting the coloring. If greater intensity and brilliancy of color are desired 85 the sand while hot is subjected to ammonia in the gaseous or aqueous forms to effect this result. If it is desired to further set or fix the coloring and increase the brilliancy thereof the sand while hot is given 90 a bath in cold liquid containing a coloring agent. This adds coloring to the sand and causes the sand to contract and the coloring in the crevices to be more pronounced.

In the production of sand having a buff, 95 brown or black color, the coloring matter is a salt or compound of iron and to produce the same I may proceed as follows: Sulfid of iron (ferrous sulfid) is pulverized and made into a paste with commercial sulfuric acid. The resulting product is diluted with water depending upon the shade of color desired, the sand being lighter in proportion to the amount of water for the dilution of the solution. Sand which has been 100 heated is soaked with the solution so as to become saturated therewith and is then dried. After this the sand may be burned in any suitable apparatus at a temperature of 100° C. or higher if desired, to increase 105 the brilliancy of the coloring. The shade of color produced and the brilliancy thereof

depends upon the temperature of the burning as well as the amount of coloring matter used.

It is not necessary except in cases where 5 a brilliant coloring is desired to heat the sand and subject it to a cold water coloring bath after it has been first heated and then given the initial cold water coloring bath, since by first heating and then giving the 10 sand a cold water coloring bath a good coloring will be given the sand.

The sand made as above described is permanent in color and may be used as an ingredient of mortar, plaster, etc., in the formation of building blocks and the like and in building and plastering walls, and it imparts its characteristic color to the molded or built product, the color being permanent, brilliant and uniform. The sand thus colored 15 is also of great commercial value in the preparation of colored roofing paper, of which the process for making will be disclosed in a separate application.

By using metallic salts of different kinds 20 other colors may be produced; for example, to produce a blue color, a copper salt is used. For this purpose pure copper may be dissolved in nitric acid and the sand is soaked in the resulting solution for several days 25 and then dried. This gives a permanent blue color which is unaffected by moisture or other influences. By subjecting this blue colored sand to the action of ammonia either in the form of gas or aqueous solution, the 30 color of the sand may be changed to green. The color of this blue sand may be deepened by burning same or heating it to a high temperature in a suitable furnace or other apparatus and by continuing the burning 35 operation to a sufficient extent a black sand 40 may be produced.

If desired black sand may be produced by the use of a saturated solution of hyposulfate of soda, by first soaking the sand in said 45 solution, the rest of the process being the same as hereinbefore described, the sand being dried, burned, subjected to ammonia while hot and the coloring fixed by giving the heated sand a cold bath.

50 Certain chemicals will intensify certain colors in the sand if the sand is pre-treated with the desired chemical before given the coloring bath; for example, hyposulfate of soda will intensify browns and reds when 55 added to the sand before it is given the coloring bath.

Various colors may be given the sand with the use of different coloring agents in the cold water bath. For example, when ammonia and hyposulfate of soda is added to 60 the water, and sand which has been colored blue is thrown into the water, the sand is changed from blue to purple.

I am aware that certain parts or steps of this process are old, for instance the mere 65 color bath treatment and subsequent burning of the sand, but it is particularly noted that I have discovered several additional steps, most notable of which is the exposure of the sand to extremes of temperature to 70 change the physical character of the sand so that it is more susceptible to color and so that the color is proof against washing out and fading.

I claim:

1. The process of coloring sand which consists in applying a coloring agent in liquid form to the sand, drying the sand, burning the sand and then giving the sand while hot 80 a cold fluid bath to fix the coloring.

2. The process of coloring sand which consists in applying a liquid coloring agent thereto, drying the sand, burning the sand and then subjecting the heated sand to ammonia.

3. The process of coloring sand which consists in applying a liquid coloring agent thereto, drying the sand, burning the sand, then subjecting the heated sand to ammonia, and then giving the sand a cold fluid bath 90 while heated.

4. The process of coloring sand which consists in heating the sand, and then giving the heated sand a cold water bath in water containing a coloring agent.

5. The process of coloring sand which consists in soaking the sand in a liquid coloring agent, drying the sand, heating the sand, and then throwing the heated sand into cold water containing a coloring agent 100 whereby the coloring of the sand is changed.

6. The process of making colored sand, which process comprises heating the sand, giving the hot sand a cold color bath, and then burning the sand.

In testimony whereof, I have hereunto set my hand at San Francisco, California, this 13th day of July, 1915.

JOHN COTTER PELTON.

In presence of—

L. BELLE WEAVER,  
A. F. SCHMIDTBAUER.